



carbon atoms and up to five in the basic molecular structure with at least two unsaturated ( $C=C$ ) groupings in the molecule. Vaporized metal bearing compounds selected from the group consisting of cyclopentadienides, biscyclopentadienyls, biscyclopentadienides, and poly-pentadienyls being utilized as the gas plating medium. The metal plating gas may be used with or without carrier gas, e.g., argon, nitrogen, as is conventional in this art.

When it is desired carrier gas may be utilized together with the dienyl metal bearing gaseous compounds, particularly where the metal vapors are to be passed through a system as when gas plating a continuously moving strip, filament or sheet. Each substrate or material which is to be plated will be heated to the proper temperature, which temperature depends upon the metal bearing dienyl compound used. Each of such metal compounds has a temperature at which it decomposes. This varies over a range, but in general temperatures between 300-1000° C. may be utilized to effect the gas plating with the dienyl metal bearing compounds.

Mixtures of these dienyl metal bearing compounds may be used to deposit a combination of the metals or alloys as desired. Further, after coating the substrate the resultant metal coated product may be annealed or heat treated as may be desired. Such annealing may also be carried out in an inert atmosphere where oxidation of the newly deposited metal coating is undesirable.

It will be understood that while the method and apparatus disclosed and described herein illustrate a preferred form of the invention and how it can be carried out, modifications obviously may be made by those skilled in the art without departing from the spirit and scope of this invention and all such modifications that fall within the disclosure and scope of the appended claims are intended to be included herein.

What is claimed is:

1. In a process of gas plating wherein the substrate to be plated is heated to a temperature sufficient to cause decomposition of a volatile metal compound brought in contact therewith, the step of bringing a gaseous metal bearing poly-enyl compound in contact with said substrate while the latter is heated above the decomposition temperature of said compound and under a non-oxidizing atmosphere to cause decomposition of the gaseous metal compound and deposition of metal onto the surface of the substrate.

2. In a process of gas plating wherein the substrate to be plated is heated to a temperature sufficient to cause decomposition of a volatile metal compound brought in contact therewith, the step of bringing a gaseous metal bearing dienyl compound containing at least three carbons in its molecular structure in contact with said substrate while the latter is heated above the decomposition temperature of said compound and under a non-oxidizing atmosphere to cause decomposition of the gaseous metal compound and deposition of metal onto the surface of the substrate.

3. In a process of gas plating wherein the substrate to be plated is heated to a temperature sufficient to cause decomposition of a volatile metal compound brought in contact therewith, the step of bringing a gaseous metal bearing poly-enyl compound in contact with said substrate while the latter is heated above the decomposition temperature of said compound and under a non-oxidizing

atmosphere to cause decomposition of the gaseous metal compound and deposition of metal onto the surface of the substrate, said poly-enyl compound being selected from the group consisting of cyclopentadienides, bis-cyclopentadienyls, biscyclopentadienides and poly-pentadienyls.

4. A process of gas plating substrate as in claim 1, wherein said metal bearing compound consists of a metal dienyl compound containing at least two carbons in the molecule.

5. A process of gas plating substrate as in claim 1, wherein said metal bearing compound consists of a metal dienyl compound containing a poly-enyl molecular structure.

6. A process of gas plating substrate as in claim 1, wherein said metal bearing compound consists of a metal diene of the metals of group Ia, IIa, IIIa, IVa, and Va.

7. A process of gas plating manganese onto a substrate which comprises heating the substrate to 500-700° C. under a non-oxidizing atmosphere, and subjecting the thus heated substrate to gaseous manganese cyclopentadienyl to cause decomposition of the manganese diene and deposition of manganese onto the surface of said substrate.

8. A process of gas plating titanium onto a substrate which comprises heating the substrate to 500-700° C. under a non-oxidizing atmosphere, and subjecting the thus heated substrate to gaseous titanium biscyclopentadienyl to cause decomposition of the titanium diene and deposition of titanium onto the surface of said substrate.

9. A process of gas plating magnesium onto a substrate which comprises heating the substrate to 500-700° C. under a non-oxidizing atmosphere, and subjecting the thus heated substrate to gaseous magnesium dicyclopentadienide to cause decomposition of the magnesium diene and deposition of magnesium onto the surface of said substrate.

10. A process of gas plating vanadium onto a substrate which comprises heating the substrate to 500-700° C. under a non-oxidizing atmosphere, and subjecting the thus heated substrate to gaseous vanadium biscyclopentadienyl to cause decomposition of the vanadium diene and deposition of vanadium onto the surface of said substrate.

11. A process of gas plating a substrate to deposit a layer of metal carbide thereon consisting of heating the substrate to 500-700° C. in a non-oxidizing atmosphere and thereafter bringing vaporous metal cyclopentadienyl in contact therewith to deposit a coating of metal carbide thereon.

12. A process of gas plating a substrate to deposit a layer of metal carbide of titanium thereon consisting of heating the substrate to 500-700° C. in a non-oxidizing atmosphere and thereafter bringing vaporous metal titanium biscyclopentadienyl vapor in contact therewith to deposit titanium carbide onto the substrate.

#### References Cited in the file of this patent

#### UNITED STATES PATENTS

2,063,596 Feiler \_\_\_\_\_ Dec. 8, 1936  
2,638,423 Davis et al. \_\_\_\_\_ May 12, 1953

#### FOREIGN PATENTS

724,799 Great Britain \_\_\_\_\_ Feb. 23, 1955